

(No Model.)

W. C. STIFF & H. B. S. BENNETT.

MANUFACTURE OF SEAMLESS TUBES.

No. 340,526.

Patented Apr. 20, 1886.



Fig. 1.



Fig. 2.



Fig. 3.



Fig. 4.



Fig. 5.

Acc'tg.  
F. A. Stiff & Co.  
Edward Stiff.

Inventor.  
Wm. C. Stiff  
Herbert B. S. Bennett  
By Knight Bros. litho

# UNITED STATES PATENT OFFICE.

WILLIAM CHARLES STIFF AND HERBERT BACHARN SOMERVILLE BENNETT,  
OF BIRMINGHAM, COUNTY OF WARWICK, ENGLAND.

## MANUFACTURE OF SEAMLESS TUBES.

SPECIFICATION forming part of Letters Patent No. 340,526, dated April 20, 1886.

Application filed November 17, 1885. Serial No. 183,123. (No model.)

*To all whom it may concern:*

Be it known that we, WILLIAM CHARLES STIFF and HERBERT BACHARN SOMERVILLE BENNETT, of the Credenda Cold-Drawn Seamless Steel Tube Company, Ledsam Street, Birmingham, in the county of Warwick, England, tube - manufacturers, have invented certain new and useful Improvements in the Manufacture of Tubes and Ordnance of Steel and Iron, of which the following is a specification.

Our invention consists of the improvements hereinafter described in the manufacture of tubes and ordnance of steel and iron.

In the accompanying drawings we have represented an example of apparatus which we employ in carrying our invention into effect.

Figure 1 is a longitudinal section, Fig. 2 is a plan, and Figs. 3 and 4 are cross-sections, of a draw bench or frame, showing a tube in position thereon; and Fig. 5 is a longitudinal section of a tapered tube in process of treatment according to our invention.

Our improvements relate to a novel method of working a cylindrical or other shaped ingot, bloom, bar, or block from which the steel or iron tube or ordnance is made.

We will describe our improvements as applied to the manufacture of steel tubes.

In the ordinary method of manufacturing seamless steel tubes a solid cylindrical ingot, bloom, bar, or block is formed by rolling or hammering or by casting, and an axial hole is made in the said ingot, bloom, bar, or block by drilling or punching, the partly-made tube being completed by rolling and drawing the same over a bulb-headed mandrel in the ordinary way, or the said hole is formed in the casting process.

According to our invention we first drill or punch a small axial hole in the solid ingot, bar, bloom, or block, and afterward enlarge the said hole to the required diameter by a drawing or other process conducted in the following manner, and we further work the said tube as hereininafter described: We fix the axially-perforated cylindrical ingot, bar, bloom, or block *a* on a bed or holder, *b*, and while the said ingot, bar, bloom, or block *a* is so fixed we enlarge the small axial hole *a'* in it by means of a bulb-headed mandrel, *c*, worked by a powerful draw

bench or machine, the rod or stem of the bulb-headed mandrel being passed through the small axial hole *a'* in the ingot, bar, bloom, or block *a* and fixed to a traveling "shoe" or "slipper," the said bulb-headed mandrel being drawn through the said block *a* in the direction of the arrow. By the action of the bulb of the mandrel *c* upon the axial hole through which it is drawn the said hole is expanded to the required diameter, the metal thus displaced expanding radially and increasing the external diameter of the ingot, bloom, bar, or block *a*, which latter is at the same time consolidated or condensed and somewhat shortened in length on account of the pressure exerted by the mandrel forcing the block *a* against the abutment *b'*. The ingot, bar, bloom, block, or partly-made tube *a*, after the hole in it has been increased in diameter to the required extent, may, by a rolling, drawing, or compressing operation, be diminished in diameter, and it may be again subjected to the action of the bulb-headed mandrel *c* in the manner before described, so as to again increase the diameter of the hole *a'*.

Instead of drawing the bulb-headed mandrel *c* through the ingot, bar, bloom, or block, the bulb-headed mandrel may be forced through the same, or it may be stationary, and the ingot, bar, bloom, or block *a* drawn or forced over the same; or both may be moved in directions toward or from each other. When forcing the bulb-headed mandrel *c* through the block *a*, it is necessary that the hole *a'* shall be sufficiently enlarged to permit of the use of a mandrel having a diameter large enough to resist the end-wise compression put upon it. When the block *a* is drawn over the bulb-headed mandrel, instead of being somewhat reduced in length, it will be slightly extended.

By the above operations the ingot, bar, bloom, or block, or partly-made tube *a* may be consolidated to any desired extent, and an axial hole of the required diameter formed in it; or, if desired, the hole may be for a part of its distance of one diameter and for another part of a larger diameter. When we make the axial hole *a'* by drilling, we effect the drilling while the ingot, bar, bloom, or block *a* is cold. When we make the axial hole by punching, we oper-

ate on the ingot, bar, bloom, or block *a* in a heated state. All the subsequent processes are performed while it is hot.

The improvements described may be applied to the manufacture of tubes and ordnance made of iron or steel.

Fig. 5 represents a partially-tapered tube suitable for ordnance in the process of manufacture. The abutment *b'* is formed with movable plates fitting into suitable guides, *b*<sup>2</sup>, and provided with holes of various sizes to suit the sizes of the bulb-headed mandrels in use, and at the same time to afford the maximum support to the end of the block *a*.

By our invention the manufacture of steel and iron tubes and ordnance is economized, and the tubes and ordnance produced are of a solidity and closeness of texture unattainable by the ordinary method of manufacture.

The production of waste metal by the drilling process hitherto employed in the manufacture of tubes and ordnance is avoided by the use of our invention.

We are aware that it is not new to confine a tube between dies, in order to prevent an increase in its external diameter and then force through its bore a mandrel having an enlarged head, whereby the diameter of the bore is increased and the metal consequently compressed between the said enlarged head of the mandrel and the confining dies; but this is not the equivalent of our invention.

Having now particularly described and ascertained the nature of our said invention and in what manner the same is to be performed, we declare that what we claim is—

1. The method, substantially as herein described, of manufacturing seamless tubes, which consists in forming a hole or bore through the ingot, bar, bloom, or block, and then passing through said hole or bore a mandrel having an enlarged head or bulb, whereby the diameter of the hole or bore, and also the external diameter of the blank being operated upon, is increased, as set forth.

2. The method, substantially as herein described, of manufacturing seamless tubes, which consists in forming a hole or bore through the ingot, bar, bloom, or block, and then forcing through said hole or bore, while the said ingot, bar, bloom, or block is heated and unconfined, against radial external enlargement, a mandrel having an enlarged head or bulb, whereby the diameter of the said bore, and also the external diameter of the blank, is increased, substantially as set forth.

W. C. STIFF.

H. B. S. BENNETT.

Witnesses to the signature of the said William Charles Stiff:

C. M. WHITE,

23 Southampton Buildings, London.

JOHN D. VENN,

9 Gracechurch Street, London.

Witnesses to the signature of the said Herbert Bacharn Somerville Bennett:

W. H. TYTHER,

12 St. Peter's Road, Handsworth, Birmingham.

W. H. HARRISON,

Parker St., Edgbaston, Birmingham.